

E. B. KIRBY.

PROCESS OF ROASTING ORES, FURNACE PRODUCTS, ORE MIXTURES, AND THE LIKE.  
APPLICATION FILED JULY 21, 1914.

1,316,726.

Patented Sept. 23, 1919.

2 SHEETS—SHEET 1.

Fig. 1.



Witnesses  
E. B. Gilchued  
L. J. Porter

Trenton  
Edmund B. Kirby  
by Thiverton & Kivis  
attorneys

E. B. KIRBY.

PROCESS OF ROASTING ORES, FURNACE PRODUCTS, ORE MIXTURES, AND THE LIKE.

APPLICATION FILED JULY 21, 1914.

1,316,726.

Patented Sept. 23, 1919.

2 SHEETS—SHEET 2.



Fig. 2.



Witnesses.

E. B. Filchus

L. J. Porter

Inventory.

Edmund B. Kirby  
by Thurston & Knis  
Attorneys

# UNITED STATES PATENT OFFICE.

EDMUND B. KIRBY, OF ST. LOUIS, MISSOURI.

## PROCESS OF ROASTING ORES, FURNACE PRODUCTS, ORE MIXTURES, AND THE LIKE.

1,316,726.

Specification of Letters Patent. Patented Sept. 23, 1919.

Application filed July 21, 1914. Serial No. 852,204.

*To all whom it may concern:*

Be it known that I, EDMUND B. KIRBY, a citizen of the United States, residing at St. Louis, in the county of St. Louis and State of Missouri, have invented a certain new and useful Improvement in Processes of Roasting Ores, Furnace Products, Ore Mixtures, and the Like, of which the following is a full, clear, and exact description.

10 This invention is a process or method of procedure by which one may quickly and definitely establish, control and regulate at all stages of a roasting operation the temperature of the individual grains of a mass 15 of material under treatment, and the chemical composition of the gases in direct contact with said individual grains, to the end that desired results may be economically and quickly produced, regardless of the 20 chemical composition of the material or its changes in chemical composition as the roast progresses.

In order to impart a clear understanding of the distinctions between the process hereinafter described and claimed and the processes heretofore used a brief review of the prior art is deemed advisable.

In the ordinary ore roasting as distinguished from sinter roasting, one much used 30 class of apparatus is such that constantly and irregularly varying gases of fuel combustion mingled irregularly with air admitted at various places is made to sweep rapidly over the surface of the crushed ore 35 which constitutes a horizontal layer several inches thick upon the hearth of a suitable furnace receptacle. This poorly mixed current of gas escapes up the chimney with only a portion of its heat, and only a portion 40 of its chemical efficiency utilized, since there has neither been opportunity for effective contact with the grains of the material, nor time for the gases to react fully with them. Each grain beneath the surface of 45 the layer is enveloped in a small volume of stagnant gases inclosed in the interstices of the material and composed of chance proportions of the overhead current and various products of the decomposition of 50 the material itself. Not only are there very wide differences in the composition of the uncontrolled gas mixtures which are in actual contact with the individual grains but there are also wide differences in the 55 temperatures of the grains themselves due to the irregular conduction of heat from

various parts of the furnace, irregularities of radiation of the flame from the furnace roof and sides upon the surface grains, heat differences in different parts of the furnace, etc. Moreover, any changes in either the temperature or chemical composition of the overhead current reach the underlying grains of the mass very slowly and irregularly.

Attempts have been made by stirring or lifting and dropping or moving the material about in the furnace to give each grain a turn-about exposure to all of these different conditions,—trying in an indefinite 70 and approximate way to keep the worst of them within limits. While these expedients have unquestionably increased the efficiency of the process, nevertheless each grain obviously has a large percentage of lost time, 75 including every period in its individual experience when it lay excluded from the roasting conditions which it should have had at that stage, and was not therefore progressing. It has also had to take its 80 turn at all the detrimental conditions present.

In muffle roasting, where gases of fuel consumption do not come in contact with the ore, but transmit their heat by conduction through the door underneath the ore and by radiation from the roof overhanging it 85 temperature changes are produced more slowly and with even great difficulty. The air supply admitted to the muffle has been 90 more or less well regulated, but this only affects the conditions to which the mass as a whole is subjected, and does not control the conditions to which the individual grains are subjected.

In those processes of roasting where the ore generates its own heat, the general mass conditions are fixed by the air admitted to different portions of the charge, but the operation is subject to the same difficulties 100 above mentioned.

In sinter roasting by the process now most commonly practised, a horizontal layer of ore mixture, which has been compounded to have the required chemical composition (if 105 the native ore did not have that composition) is first ignited by direct contact with a flame or with burning fuel; and a current of air is thereafter drawn or blown through it to support the combustion. Generally 110 speaking, this entire layer is progressively subjected to the same fixed and unchange-

able conditions without any power of regulation. The action is like that of a fire running through a hay field or through a fuse which has been carefully composed or prepared for it.

With the old processes and the apparatus through which they were practically carried into effect, mass conditions only were controlled, and these were controlled only imperfectly at best. No attempt even has ever been made for definitely establishing and controlling and promptly varying conditions to which the individual grains were subjected. Ore roasting as heretofore practised has not heretofore been nearly as efficient or economical as it should be in any case. Additionally it has been known that ore roasting to be most efficient and most satisfactory required many refinements in the treatment of the ores, such as confining sulfatization within certain desired limits, avoiding the formation of certain insoluble ferrites, and also the sintering of ore mixtures containing other than certain proportions of sulfur, etc., these refinements having been either too expensive to practice or wholly impossible.

In the process herein described and claimed a charge of the material comminuted to the required fineness is confined in a receptacle wherein it is substantially isolated from any externally generated heat or gas, save those of the current to be described, and a current of prepared gases having certain definite composition known to be required at the time with the particular ore under treatment to produce best results, is preheated to the definite temperature required but is never heated to such temperature as that in view of the other conditions the ore will be caused to or allowed to ignite or break into conflagration; and this gas so preheated to the required temperature, and having the required chemical composition is caused to flow through the interstices of the comminuted ore and in intimate contact with the individual grains thereof until desired results are attained; and to whatever extent may be necessary or desirable the chemical composition of the gas, and its temperature may be definitely varied at different stages of the roasting operation.

Of course, to carry out said process in any practical way, some apparatus is required, and such an apparatus, and various modifications thereof are fully described in a copending application.

In the drawing Figure 1 is a plan view somewhat diagrammatic in character of an apparatus suitable for the practice of this process. Fig. 2 is a longitudinal vertical section through one end of the furnace showing the means by which the comminuted material is suitably confined and the means by which the preheated and properly com-

pounded gas current is delivered into and withdrawn from the comminuted ore.

The apparatus comprises a number of appliances operatively connected. It is shown in Fig. 1 in a complete form adapted for use with all kinds of ores and for the production of all possible desirable effects upon them, as required by the process herein described and claimed. It includes a furnace or receptacle 1 for holding the comminuted ore in such a way that the current or blast of prepared and preheated gases may be caused to flow through the interstices of the ore. It also includes a pressure fan or blower 2 for forcing the prepared gases into said receptacle; a hot blast stove 3 for preheating the prepared gas, a vacuum fan or blower 4 for withdrawing the gas from said receptacle, an incoming gas main 7, the outgoing gas main 8, a separating device 5 for collecting the dust and fume in the outgoing gas current; the chimney 6 into which said outgoing main discharges, and suitable pipes, valves, etc., as hereinafter described.

All parts of this apparatus, except the furnace 1 and the component parts thereof to be described, consists of standard or well known appliances, each of which is constructed in a great variety of designs. I do not limit myself to any particular form or design of any of these individual parts, selecting whatever suitable device is most readily obtainable at a satisfactory price. Moreover, with many ores all of the above mentioned appliances are not required; for example, it is self evident that with some ores either the pressure fan or the vacuum fan alone might be made to move the current.

The hot blast stove 3 is of the pipe class,— that is to say, the stove includes a combustion chamber 3<sup>a</sup> connected with a chimney 13, an oven 3<sup>b</sup>, and suitable pipe coils 10 in the oven. These pipe coils are connected in series with the gas supply pipe 11 which leads away from the blast fan 2, and with the incoming gas main 7. The various coils are connected with a by-pass pipe 12 which connects pipe 11 with the gas main 7. In the piping are valves 11<sup>a</sup>, 12<sup>a</sup>, 3<sup>c</sup>, 3<sup>d</sup>, 3<sup>e</sup>, by the manipulation of which the blast current may be by-passed as desired from part or all of the pipe coils. As a further means of regulation the heating of the oven 3<sup>b</sup> may be governed by the short circuiting damper 3<sup>f</sup> between the fireplace 3<sup>a</sup> and the chimney 13.

The inlet pipe 14 of the blast fan 2 is connected with several pipes, through which it draws such gases as are necessary for producing the particular gas mixture required. The pipe 15 is that through which air may be drawn, and it contains a gaged valve 15<sup>a</sup> by which to regulate the size of the orifice through which the air must flow, and thereby to regulate the rate of flow. 16 repre-

sents a pipe (and there may be any number of pipes of this sort) connected with the inlet pipe 14, and is to be connected with a source of the particular kind of gas which 5 may be required in the gas mixture, and each of these pipes will contain a gaged valve 16<sup>a</sup> by which to regulate the rate of flow of said gas from said container into pipe 14. 17 represents a pipe which connects pipe 14 with pipe 18 through which the 10 hot exhaust gases from furnace 1 are led to and discharged into chimney 6. The gaged valves 17<sup>a</sup> and 18<sup>a</sup> provide means by which to determine what part of the said hot exhaust gases are allowed to go into the chimney, and what shall be allowed to go into inlet pipe 14. 19 represents a pipe for connecting the inlet pipe 14 with the combustion chamber 3<sup>a</sup> of the hot blast stove, and it 15 contains a gaged regulating valve 19<sup>a</sup>.

As many of these gas supply pipes with regulating valves may be provided as may be required, and they may be connected with suitable sources of the desired gases. With 20 the construction shown, however, provision is made for preparing, as required for use and immediate delivery to the fan, a gas mixture made up of measured and therefore properly proportioned parts of air, the hot 25 gaseous products of fuel combustion from the stove combustion chamber containing CO<sub>2</sub>, the hot exhaust gases discharged from the ore roasting furnace, and any other needed gas; and for most ore roasting operations, desired results can be obtained by 30 mixtures made up of suitable proportions of these gases, provided that, as they pass from the fan to the inlet main 7, they are pre-heated to the required temperature.

40 The furnace is preferably a rectangular receptacle without a top. In it are two series of gas conduits which, when said chamber is filled with comminuted material, will be buried therein. One group of these conduits will be connected with the inlet main 7, and will hereinafter be referred to as incoming gas conduits, while the other group of conduits will be connected with the exhaust main 7 and will be hereinafter referred to as outgoing gas conduits. The 45 conduits of one group must be arranged in such juxtaposition to those of the other group that the incoming gas passing through suitable properly distributed gas 50 passages in the incoming gas conduits will flow through the interstices of the surrounding mass of material in the furnace receptacle, and thence into the outgoing gas conduits. Various forms of gas conduits may 55 be employed, and the openings or passages for the discharge reception of gas may be of various forms.

As shown in Fig. 2, however, each of the 60 incoming gas conduits 25, and each of the outgoing gas conduits 35 is a substantially

vertical hollow leaf or partition, extending across the furnace receptacle from side to side and from the bottom to the top thereof. There may be as many of these partition-conduits as are required. The incoming 70 partition conduits are arranged alternatively with the outgoing conduits and in parallel and rather close relation thereto, so that they divide the space within the furnace receptacle into numerous ore cells, and 75 divide the ore mass into a number of substantially vertical thin sheet like layers which respectively fill said cells. The thickness of each vertical ore sheet, that is to say, the distance between adjacent partition conduits must be such that the current of gas 80 can flow across this space through the interstices of said sheets of comminuted ore.

For a more complete description of an apparatus and the various modifications of an apparatus suitable for the practice of this process with various specific kinds of ore, reference may be had to the companion application hereinbefore referred to. It is perhaps sufficient for the present to say that 85 these partition conduits may be made of any material which is best adapted to the nature of the gas employed and the temperatures to which they are subjected. These partition conduits may have a large 90 number of gas passages 33 made through their opposed walls, and these gas passages may have any particular form and be of any particular size best adapted to the particular ore to be treated. The upper and 95 lower parts of these partition walls should be imperforate. In charging the furnace, inert material, such as ore which has already been roasted, should be packed between the imperforate lower part of these 100 partition conduits in sufficient quantity to serve as a seal, preventing the downward escape of gas. Next above this inert material and between the perforated walls of the partitions will be packed the unroasted 105 comminuted ore or other material to be treated. Above this and between the imperforate upper parts of the partitions will be packed a sufficient quantity of material 110 which may be unroasted ore, to act as a seal to prevent the escape upward of said gas. During the roasting operation the ore sheets in the several ore cells between partitions will be held by suitable gates 57 at 115 the lower ends of said ore cells.

Before roasting any ore or other material according to the herein described process and with the above described apparatus or any other suitable apparatus, one should first determine what combination of gases 120 will produce in the most satisfactory degree the desired results upon that particular ore, and at what temperature these results will be produced in the more satisfactory degree, and whether, as the composition of 125

the ore under treatment is varied by the treatment, it is desirable to change either the components of the gas current or its temperature, and to what extent and how. 5 These things being definitely determined, the ore or other material, comminuted to the proper degree, is charged into a receptacle in a comparatively thin layer, care being taken to isolate the charge therein 10 from any externally generated heat, save the flameless heat which is delivered thereto by the preheated gas current. Then the compounded gas containing definite proportions of the required component 15 gases, and preheated to the determined temperature, is caused to flow swiftly through the interstices of the charge and in intimate contact with the grains thereof, thereby producing, uniformly and quickly, 20 those results upon said charge which said gas, so preheated, is adapted to produce, and some of the gas after passing through the charge may be recirculated through it in order to obtain its full effect; this re- 25 circulation being carried to any extent that is found desirable.

The definite composition of the gas current and the definite temperature to which it is preheated are under perfect control 30 independently of each other and are regulated by being immediately varied as required during the progress of the roasting operation. Any adjustment of temperature made by the stove by-pass valves or of 35 composition made by the gas supply valves, is felt within a few seconds and with substantial uniformity by every individual grain of the charge.

Both the temperature of the current and 40 the percentages of its active components are regulated to the definite points required within whatever limits of accuracy may be necessary. The temperature regulation is guided by suitable pyrometers placed in the 45 gas current and also in the charge of material. The regulation of composition is guided by any suitable devices of the class known in the arts for indicating or determining either continually or at intervals 50 the percentage of any gaseous component to be governed.

As one illustration of the many new results which may be accomplished by this definite and perfect regulation, there are 55 ores, for example, which, when the roasting operation is concluded, should be delivered in a sintered instead of a comminuted condition, but which contain an excess percentage of oxidizable components over that required 60 for sintering. In the treatment of such ores the percentage of free oxygen in the gas current should be kept low so that this excess of oxidizable components will be slowly oxidized. If it were not, the great heat de- 65 veloped internally by the rapid oxidation

of these components might produce undesirable changes in the ore. The percentage of free oxygen in the gas current may be kept low by diluting the air, to whatever extent may be necessary, by including in the 70 gas mixture air with more or less of the hot exhaust gas which has passed through the ore, or with more or less of the gaseous products of combustion from the stove combustion chamber. By as much as these may be 75 added, they supplement the hot blast stove in preheating the gas current, and thereby reduce the cost of so preheating said gas.

When, in the described treatment of this ore the excess of the oxidizable components 80 thereof have been slowly oxidized, the ore may be caused to quickly sinter by definitely increasing the percentage of free oxygen in the gas current, and this sintering may be assisted by also increasing the pressure 85 of said gas as it flows through the interstices of the charge.

I believe that no method of ore roasting has heretofore been suggested by which one could subject all of the individual grains 90 of the material to be treated at substantially the same time to substantially uniform conditions, or could make those conditions precisely such as were most efficient for the time being with any kind of ore or could 95 almost immediately definitely alter and regulate those uniform distributed conditions as required for the production of desired results in the highest degree.

In cases where the ore becomes sintered 100 or agglomerated in roasting and the resulting sheet of sintered ore tends to adhere to the walls of the furnace or to the side of the outgoing conduit or to choke its apertures, such adhesions or choking may be prevented by so charging as to deposit a thin layer of non-adhering material along the face of the ore sheet which is in immediate contact with said walls or said outgoing conduit. 105

Such non-adhering material may, for instance, be the fines returned from the roasted product or fluxes which are to be used with it afterward, or on the other hand it may be the more infusible components or the coarser lumps of the charge itself separated from it temporarily for this purpose. 115

Having described my invention, I claim:

1. The process of roasting ores, furnace products, ore mixtures and the like which consists in confining the material in a suitable comminuted condition in a thin sheet in a receptacle; in causing the passage through the interstices of said material and in intimate contact with the individual grains thereof of a compounded gas made up of definite proportions of the gaseous components required, which compounded gas is preheated to the definite temperature required before it is discharged into said 120

material, in restricting the percentage of oxygen in said mixture for a time to such a degree that sintering of the material will not take place; and in, at the proper time, 5 suddenly increasing the percentage of oxygen in the gaseous compound to a degree such as will induce sintering.

2. The process of roasting ores, furnace products, ore mixtures and the like which 10 consists in placing the charge in a receptacle where it is substantially isolated from any heat or gases save those of the current to be described; and in causing a prepared current of gases to flow through the interstices 15 of the charge and in intimate contact with

the individual grains thereof and in pre-heating said current to the definite temperature required before it comes in contact with the charge and in having said current include for recirculation a greater or less 20 proportion of the outflowing current from the charge.

In testimony whereof, I hereunto affix my signature in the presence of two witnesses.

EDMUND B. KIRBY.

Witnesses:

E. L. THURSTON,  
L. I. PORTER.